

Feb. 13, 1951

E. J. ROEHL ET AL

2,541,721

PROCESS FOR REPLENISHING NICKEL PLATING ELECTROLYTE

Filed April 22, 1948



## UNITED STATES PATENT OFFICE

2,541,721

PROCESS FOR REPLENISHING NICKEL  
PLATING ELECTROLYTE

Edward Judson Roehl, Little Silver, and Andrew Wesley, Plainfield, N. J., assignors to The International Nickel Company, Inc., New York, N. Y., a corporation of Delaware

Application April 22, 1948, Serial No. 22,727

11 Claims. (Cl. 204—49)

**1** The present invention relates to a process for electrodepositing nickel employing an insoluble anode wherein the nickel content and acidity of the electrolyte employed are maintained substantially constant and, more particularly, to a feasible process for nickel plating with an insoluble anode wherein the nickel content and acidity of the nickel plating electrolyte are maintained substantially constant by electrolytic means and the electrolyte is maintained in condition to permit the production of sound nickel electrodeposits therefrom.

It has been recognized in the art that insoluble anode processes for electroplating nickel offer distinct advantages in many fields. For example, in the plating of steel strip and wire, the electroforming of fine screen material and parts of intricate or irregular shape, plating the inside of tubes, etc., it is important that the distance separating anode from cathode be kept substantially constant and this is most readily accomplished by employing anodes which are substantially insoluble in the plating bath. As recognized by those skilled in the art, the metal ions for plating must be provided by the plating bath as substantially no metal ions are supplied by the anode in the insoluble anode plating process. This results in the disadvantage that the bath used for plating with an insoluble anode becomes depleted in metal ion content and, since the metal ions plated out are replaced by an equivalent amount of hydrogen ions by electromechanical reactions, the acidity of the bath increases. Due to the combination of these factors, the bath eventually becomes unsuitable for further plating unless steps are taken to replenish the metal ion content and to decrease the acidity.

In the plating of copper using insoluble anodes, the copper plating solution can be replenished simply by passing it over copper scrap, etc., as the solution reacts with the copper to increase the copper content and decrease the acidity of the solution. However, nickel presents an entirely different problem and, when replenishment of a depleted nickel electrolyte is attempted in a similar manner, the results are unsatisfactory and the method impracticable. For example, the rate of corrosion of the nickel scrap, etc., in the electrolyte is very low and, in addition, nickel has a strong tendency toward passivity in the electrolyte, particularly the chloride-free electrolyte. These and other factors require that the volume of solution and surface area of scrap used in the replenishing

system be so impractically large that no satisfactory method employing this principle has yet been devised. Other methods have been tried or proposed for the replenishment of depleted nickel electrolytes, for example, treatment with basic nickel compounds such as nickel carbonate and the use of an electrolytic replenishing system employing porous diaphragms in the plating baths. However, these methods are expensive and difficult to maintain. Thus, in the treatment with a basic nickel compound, difficulties are encountered in continuous operation and there is a tendency for the nickel content and pH of the plating electrolyte to fluctuate. **15** In the porous diaphragm method, power costs are high and it is difficult to maintain the diaphragm in good operating condition. Although many attempts have been made to remedy these and other shortcomings, none, as far as we are **20** aware, was entirely successful when carried into commercial practice.

Thus, a definite need exists in the art to provide a successful method whereby nickel electrodeposits can be produced employing an insoluble anode, and at the same time, the nickel ion content and acidity of the electrolyte are maintained substantially constant in ranges where the production of sound nickel deposits at a satisfactory rate is feasible.

**25** It is an object of the present invention to provide a process for electrodepositing nickel from a cell having an insoluble anode wherein the nickel content and pH of the electrolyte are maintained substantially constant.

It is still another object of the present invention to provide a method for replenishing the nickel content and maintaining the acidity of the electrolyte used in electrodepositing nickel employing an insoluble anode.

**35** It is a further object of the present invention to provide an electrochemical method for simultaneously providing a supply of nickel ions to and diminishing the acidity of a nickel plating electrolyte.

**40** It is a still further object of the present invention to provide a method for efficiently dissolving nickel electrolytically.

It is another object of the present invention to provide a method whereby electrolytic nickel may be dissolved electrolytically at high efficiency in a chloride-free nickel plating bath and, at the same time, to maintain the bath in condition that satisfactory nickel electrodeposits may be produced therefrom at feasible rates of deposition and over long periods of time.

Other objects and advantages of the present invention will become apparent from the following description taken in conjunction with the drawing which depicts schematically an embodiment of the invention.

Broadly stated, the process of the invention comprises electrodepositing nickel at a plating cathode by passing a direct current through an acid aqueous nickel sulfate plating electrolyte from an insoluble anode to the plating cathode (said insoluble anode and said cathode being at least in part immersed in said electrolyte), replenishing the nickel content of depleted plating electrolyte by passing a direct current therethrough between electrodes having a nickel surface exposed to the electrolyte at a current density of about 1 to 25 amperes per square foot of effective anode surface exposed to the electrolyte, reversing the direction of said direct current at intervals of about 1 to about 50 seconds, and electrodepositing nickel from the thus-replenished electrolyte. The reversal of direct current flow during the replenishing operation will usually be repeated as often as required to replace nickel removed from the electrolyte in prior electrodeposition and to provide the nickel concentration required for further electrodeposition of nickel from the replenished electrolyte. In practice, the electrolyte can be transferred from the electroplating unit to the replenishing unit and returned either at a continuous or intermittent rate of transfer.

It is critical that three separate operating factors be met in carrying out the present invention. That is, in the replenishing operation the nickel surface of the anode must be maintained in an active condition and there must be an economically feasible difference between anode efficiency and a lower cathode efficiency, while in the plating operation an opposing high electroplating efficiency, e. g., cathode efficiency, must be maintained. Inability to meet any one of these operating factors would vitiate the entire process, and the present invention resides in the unexpected discovery of a set of conditions which enables satisfying these critical factors simultaneously. These factors are met simultaneously by the conditions defined herein. Thus, the activity of the nickel surfaces of the anode and the differential between the higher anode efficiency and lower cathode efficiency is maintained during the replenishing operation by employing the reversed direct current at the current densities and for the time intervals set forth herein and by employing a nickel sulfate plating electrolyte substantially devoid of chloride. The high electroplating efficiency is simultaneously maintained by employing a nickel sulfate plating electrolyte such as described herein.

In practice, the aqueous acid nickel sulfate electrolyte employed in the process contains or is comprised essentially of about 100 to about 400 grams of nickel sulfate per liter of electrolyte, buffered with about 10 to about 50 grams of boric acid per liter, said electrolyte having a pH of about 0.75 to about 3.5, a temperature of about 100° to about 160° F., and being substantially devoid of chlorides, i. e., containing not more than about 1 gram per liter of chloride ion, preferably not more than about 0.01 to 0.1 gram per liter. Preferably, the electrolyte contains about 250 to 350 grams per liter of nickel sulfate, about 20 to 40 grams per liter boric acid, and has a pH of about 1 to 2. It is to be pointed out that the object of the replenishing operation is to main-

tain the composition of the electrolyte during the electroplating operation within the aforesaid ranges in order that plating may be satisfactorily carried out for long periods of time. The current density employed in the electroplating operation

5 may be from about 25 to about 2000 amperes per square foot. By way of example, it may be said that an aqueous electrolyte containing or comprised essentially of about 300 grams per liter of nickel sulfate and about 30 grams per liter of boric acid, operated at a pH of about 1.5 and a temperature of about 130° F., has been found to be satisfactory and to give optimum overall efficiency for the system in a closed circuit of separate electroplating and replenishing operations.

Control of electrolyte pH is also a critical aspect of the process as a whole because it has been found that when the pH is lower than about 0.75 the efficiency of electroplating is impractically low, while when the pH is higher than about 3.5 the net gain of nickel dissolved in the replenishing operation is impractically low.

20 The nickel electrodes employed in the replenishing operation are preferably made of electrolytic nickel, although the nickel electrodes can be any anode material which will supply dissolved nickel to the electrolyte when it acts as anode during the replenishing operation, e. g., cast or wrought nickel anodes, and which does not introduce harmful amounts of contaminants into the nickel plating electrolyte.

25 A feature of the present invention is that a satisfactory regenerative plating system for nickel plating with an insoluble anode is provided in which an electrolytic replenishing operation has been devised wherein nickel is dissolved anodically at a favorably higher rate than it is deposited cathodically, i. e., wherein the anode efficiency is favorably higher than the cathode efficiency. When this condition is achieved, the function of the replenishing operation to supply nickel ions and to decrease the acidity in the plating electrolyte which has been depleted in nickel ions and has become more acid in the 30 plating operation is realized. In the present invention, this has been provided by control of critical features affecting the replenishing operation and including the reversal of the flow of the direct current applied between the electrodes employed in the replenishing operation, the time cycle of current reversal, the current density effective upon the electrodes, the pH and composition of the electrolyte, etc. It has been found that reversal of the direct current is essential and that the direct current must be reversed at intervals of from about 1 to about 50 seconds (cycles of about 2 to about 100 seconds), preferably at intervals of about 3 to 7 seconds e. g., 5 seconds. It is important to avoid reversing intervals shorter than about 1 second (for example, as represented by 60-cycle alternating current) or longer than about 50 seconds, as it has been found that both conditions produce low electrochemical efficiency in the replenishing operation with the result that the net gain of nickel dissolved becomes too low for successful operation. In addition to the foregoing, it is critical that the net current density applied on each electrode in each direction of current flow be maintained within the aforementioned range of about 35 1 to about 25 amperes per square foot in the replenishing operation, preferably about 5 to 15 amperes per square foot, e. g., 10 amperes per square foot, because at current density values below the minimum the rate of dissolution of

nickel becomes impractically low, while at current density values above the maximum the rate of deposition of nickel in the replenishing operation approaches and may even exceed the rate of dissolution of nickel therein, with the result that the net gain of nickel dissolved in the electrolyte decreases below practicable limits. It is preferred that the time intervals and current density in the replenishing operation be so chosen that the same number of ampere hours per square foot is alternately applied on the cathode side in each direction of current flow, e. g., the same current density and the same time interval for each reversal of current flow, as otherwise one set of electrodes would dissolve faster than the other set or might even grow at the expense of the other. In addition, some difficulties might be encountered by way of growths on one set of electrodes which might produce short circuits, particularly when the electrodes are closely spaced. From a practical standpoint, it is desirable to replace both sets of electrodes at the same time and to employ electrodes of substantially the same area.

As indicated hereinbefore, it is important that conditions in the replenishing operation be such that the rate of solution of nickel at the anode is favorably higher than the rate of deposition of nickel at the cathode, i. e., the anodic efficiency of the operation must be higher than the cathodic efficiency. Thus, anode efficiencies should be at least as high as about 50% and may be as high as about 100% while cathode efficiencies may be as low as about 25% or 30%, but should not be over about 70%. The difference between anode and cathode efficiencies may be about 10% to about 70% and preferably should be about 50% or more.

The process of the present invention is preferably carried out using a substantially chloride-free nickel plating bath, i. e., a bath containing less than 0.1 gram of chloride ion per liter. However, amounts of chloride up to about 1 gram per liter, e. g., about 0.01 to 1 gram per liter, do not adversely affect operation of the process. It has been found that if the chloride ion content substantially exceeds this amount, the efficiency of the replenishing operation with respect to net gain of nickel dissolved is markedly reduced and other difficulties may be encountered.

It has been found that the electrochemical efficiency of the replenishing operation is highest when both the current density and the pH of the electrolyte are low. If either of these factors approaches the permissible maximum recited herein it is preferred that the other factor be maintained near the minimum recited herein. For example, when replenishing is carried out at a current density of 25 amperes per square foot it is preferred that the pH of the electrolyte be about 1 or less. If the current density is only 1 ampere per square foot, then the pH of the electrolyte can be as high as about 3.5. Various means may be employed to insure meeting the various requirements set forth hereinbefore. For example, in a case where the current efficiency with respect to net gain of dissolved nickel in the replenishing operation is the same as the current efficiency with respect to deposition of nickel in the plating operation and the replenishing operation is conducted with a current density of 10 amperes per square foot and the plating operation is operated at 50 amperes per square foot, the electrode area for each set of electrodes in the replenishing operation should be at least about five times as great as the cathode area in

10

15

20

25

30

35

40

45

50

55

60

65

the plating operation if it is desired to maintain substantially equal rates of depletion and replenishment of nickel in the system. By observing any changes in the nickel ion content and/or pH of the electrolyte, it is possible to maintain control of the overall performance of the system. For example, a drop in nickel content or increase in acidity indicates that nickel is being depleted more rapidly in the plating operation than it is being dissolved in the replenishing operation, while an increase in nickel content and decrease in acidity indicates the opposite. Control measures such as increasing the electrode area in the replenishing operation can be employed to maintain the nickel content and acidity of the electrolyte substantially constant when the process embodying the invention is in operation. Other control measures may also be employed. For example, the rate of nickel dissolution in the replenishing operation can be increased or decreased by respective increases or decreases in current density without changing conditions in the plating operation. Likewise, the current density in the plating operation can be controlled to increase or decrease the rate of nickel depletion in the electrolyte, etc.

It is to be noted that small amounts of impurities which do not interfere with the working of the plating operation can be tolerated in the nickel sulfate electrolyte. In order to conform with accepted standards for good nickel plating practice, the impurities in the electrolyte can be tolerated within the following ranges:

|                     | Grams per liter  |
|---------------------|------------------|
| Iron                | 0.0008 to 0.15   |
| Copper              | 0.0012 to 0.04   |
| Zinc                | 0.005 to 0.05    |
| Lead                | 0.00005 to 0.002 |
| Aluminum            | 0.002 to 0.06    |
| Hexavalent chromium | 0.005 to 0.01    |

If calcium is present, it may be included in amounts from about 0.002 gram per liter up to the concentration at which  $\text{CaSO}_4$  precipitates.

Suitable equipment for carrying out the invention comprises an electroplating unit comprising an insoluble anode and a cathode, and having a direct current supply; a replenishing unit comprising one or more nickel electrodes of each polarity and provided with a direct current supply having current reversing means; means for circulating electrolyte between the two units (e. g., pumps, stirrers, etc.); and conventional auxiliary equipment such as heating means, etc., for controlling conditions, etc., in the equipment. The electroplating unit and the replenishing unit may be contained in separate cells (or tanks) or in separate compartments of the same cell (or tank), or may even be contained in the same compartment.

In order that those skilled in the art may have a better understanding of the present invention, the following illustrative example is given describing the operation of a regenerative plating system for plating nickel using an insoluble anode.

#### EXAMPLE

A recirculating plating and replenishing system illustrated schematically in the drawing was set up comprising a plating tank 1 and a replenishing tank 2 of approximately equal size connected to permit flow of solution from one to the other 3 and 4, a pump for circulating the electrolyte from one tank to the other 5 and back again 6,

stirring devices in each tank and heating means 7 to maintain the electrolyte temperature. The plating tank was provided with a cathode 8 and an insoluble anode 9 and the replenishing tank was provided with a row of five equal electrolytic nickel electrodes 10 disposed in face-to-face relationship and having alternate electric polarity. In this manner, four sets of electrode surfaces of equal effective area and of opposite polarity were provided. Each tank was provided with an independent direct current power supply 11 and 12, that to the replenishing tank being provided with current reversing means 13. A chloride-free aqueous nickel sulfate plating bath was established containing about 300 grams of nickel sulfate per liter of electrolyte (72.5 grams per liter of nickel) and 30 grams of boric acid per liter. The bath was purified according to standard procedure. Thereafter, the bath pH was adjusted to 1.3 and the temperature was adjusted to and maintained at about 130° F. for the duration of the run, and the electrolyte was circulated between the tanks at a rate equivalent to a complete circulation of the electrolyte every 2 hours. A run of 28 hours duration was then made during which the current density in the plating cell was maintained at about 40 amperes per square foot and that in the replenishing cell was maintained at about 10 amperes per square foot. The direct current flow in the replenishing cell was reversed at 5-second intervals. The effective area of one set of electrodes (effective area of each polarity) in the replenishing cell was about 8.67 times the cathode area in the plating cell. At the end of the run, the electrolyte pH was 1.2 and the nickel content was 70.7 grams per liter. The metal deposit obtained during the run was stripped from the cathode and machined into tensile test strip specimens. Results of tests on these specimens are shown in Table I, together with comparative results obtained on nickel electrodeposited from a standard Watts-type bath using soluble anodes.

TABLE I

*Test results on electrolytic nickel from sulfate bath*

| Thickness,<br>in. | Hardness,<br>VHN <sup>1</sup> | Tensile<br>Strength | Percent Elongation in— |     |       |
|-------------------|-------------------------------|---------------------|------------------------|-----|-------|
|                   |                               |                     | 1"                     | 1½" | 2"    |
| .033              | 167                           | 76,000              | 25                     | 20  | 18    |
| .033              | 162                           | 78,000              | 29                     | 22  | 19    |
| .036              | 160                           | 77,000              | 30                     | 22  | 19    |
| .034              | 148                           | 68,250              | 24                     | 20  | n. d. |

n. d.=not determined.

<sup>1</sup> Vickers hardness number—10 kg. load.

<sup>2</sup> Test results on deposit obtained from standard Watts-type bath operated at 170° F., pH 1.0, a cathode current density of 50 amperes per square foot, containing 325 grams per liter nickel sulfate, 45 grams per liter nickel chloride and 30 grams per liter of boric acid.

As indicated in the foregoing example, when the process embodying the invention is employed in the plating of nickel from a sulfate electrolyte using a plating cell having an insoluble anode, the electrolyte composition can be maintained substantially constant over long periods of time. In addition, the electrodeposited metal obtained thereby compares favorably in tensile strength and ductility to metal deposited from a chloride-containing bath (such as a Watts-type bath) using a soluble anode.

The present regenerative insoluble anode electroplating process is adapted to the production of electroformed articles and the like. Operation of

the present process is attended by numerous practical advantages. Thus, no anode bags are needed in the plating operation; undesirable contaminants can readily be excluded or eliminated from the electrolyte; close control of the anode to cathode distance in the plating operation can be maintained; electrodes may be closely spaced in the replenishing operation; nickel is supplied to the electrolyte from nickel electrodes which can be of high purity, e. g., electrolytic nickel, and which operate at good activity; good control of the process is readily maintained; standard equipment may be readily adapted to the process; and the cost of the process is substantially lower than the cost for any known insoluble anode plating process, comparing favorably even with soluble anode plating processes.

It is to be pointed out that insoluble anodes made of lead preferably should not be used during the electroplating operation wherever slight lead contamination would be harmful to the mechanical and/or physical properties of the resulting electrodeposited article. For example, although articles made in the plating operation using lead anodes have satisfactory strength and ductility in the as-plated condition, these articles tend to become weak and brittle upon annealing. More preferred insoluble anodes may be fashioned from platinum or from platinum-base alloys containing other platinum-group metals. Thus, platinum alloys containing iridium up to 30% or rhodium up to 40% or ruthenium up to 15% may be used. As previously indicated, pure platinum may also be used, but if other platinum-group metals are present they will be included in amounts exceeding about 0.01% each. Not only may platinum-base alloys containing palladium be employed but palladium-base alloys containing platinum will also give acceptable results. Other precious metals, such as gold, also give acceptable results. Base metals having corrosion-resistant properties similar to tungsten may also be employed as well as tungsten. Among the non-metallic materials, magnetite may be mentioned as a suitable insoluble anode material. Graphite anodes produce acceptable nickel electrodeposits, but this material is not preferred because of its tendency to gradually disintegrate when used as anode in the electrolyte. The term "insoluble anode" is used herein in its conventional sense and means a conducting material which is either completely insoluble or which corrodes in the bath at such a low rate that its replacement is economical and practical and that it does not build up harmful soluble or insoluble impurities in the bath at an excessive rate.

It will be recognized from the foregoing that the electrolyte should be subjected alternately to electroplating and replenishing operations. This will normally require circulating the electrolyte between the electroplating and replenishing units at a rate sufficient to maintain the nickel concentration in the replenished electrolyte at a level suitable for further electroplating in the electroplating unit. The proper rate of electrolyte transfer between these units necessary to achieve this result will vary with each application since this rate depends upon many variable factors such as the volume of the plating electrolyte, rate of extraction of nickel from the bath in the plating operation, rate of replenishment of nickel in the replenishing operation, etc. As indicated hereinbefore, these factors are controlled by the current densities employed in both the electroplating and replen-

ishing operations, the number of current reversals during the replenishing operation and the intervals at which the current is reversed in the replenishing operation and the pH and composition of the plating bath.

As indicated hereinbefore, any anode materials which will supply dissolved nickel to the electrolyte when acting as anode therein and which do not introduce harmful amounts of impurities such as iron, zinc, etc., into the electrolyte may be employed as electrodes in the replenishing operation, but it is preferred that electrolytic nickel anodes be used. As those skilled in the art know, electrolytic nickel is a high purity nickel containing more than 99% nickel (including a small amount of cobalt which is usually less than 1%).

Other satisfactory soluble anodes (i. e., anodes which show good activity and which dissolve readily in the nickel electrolyte) which may be employed in the replenishing operation are cast and wrought nickel anodes usually having analyses within the following ranges:

|                                | Range     | Specific Examples |         |
|--------------------------------|-----------|-------------------|---------|
|                                |           | Cast              | Wrought |
| Nickel (including cobalt)..... | 99 to 100 | 99.33             | 99.6    |
| Iron.....                      | 0 to 0.1  | 0.054             | 0.05    |
| Copper.....                    | 0 to 0.1  | 0.02              | 0.045   |
| Sulfur.....                    | 0 to 0.02 | 0.006             | 0.005   |
| Carbon.....                    | 0 to 0.5  | 0.24              | -----   |
| Silicon.....                   | 0 to 0.5  | 0.26              | 0.01    |

Although the present invention has been described in conjunction with preferred embodiments, it is to be understood that modifications and variations may be resorted to without departing from the spirit and scope of the invention, as those skilled in the art will readily understand. Such variations and modifications are to be considered within the purview and scope of the invention and the appended claims.

We claim:

1. The process for electrodepositing nickel which comprises establishing an aqueous nickel plating electrolyte essentially comprised of about 100 to 400 grams per liter of nickel sulfate, about 10 to 50 grams per liter of boric acid, substantially devoid of chloride ions, having a pH of about 0.75 to 3.5 and a temperature of about 100° to 160° F., electrodepositing nickel from said electrolyte in an electroplating unit having a source of direct current, at least one insoluble anode and at least one cathode by passing a plating current from said direct current source through said electrolyte from said insoluble anode to said cathode to electrodeposit nickel at said cathode, flowing said electrolyte to a replenishing unit comprising a source of reversible direct current in electrical connection with a plurality of nickel electrodes, substantially replenishing the nickel content of said plating electrolyte by passing therethrough between said electrodes direct current from said source of reversible direct current at a current density of about 1 to 25 amperes per square foot while repeatedly reversing the direction of said direct current at time intervals of about 1 to 50 seconds to obtain a net gain of nickel dissolved from said electrodes, flowing the thus-replenished electrolyte to an electroplating unit and electrodepositing nickel from the thus-replenished electrolyte.

2. The process according to claim 1 wherein

the aqueous nickel plating electrolyte is essentially comprised of about 250 to 350 grams of nickel sulfate per liter of electrolyte, about 20 to 40 grams per liter of boric acid, and has a pH of about 1 to 2, wherein the direct current in the replenishing unit flows at a current density of about 5 to 15 amperes per square foot and wherein the direction of said current is reversed at time intervals of about 3 to 7 seconds.

3. The process according to claim 2 wherein the current in the replenishing unit flows at a current density of about 10 amperes per square foot and wherein the direction of said current is reversed at intervals of about 5 seconds.

4. The process according to claim 3 wherein the aqueous nickel plating electrolyte is essentially comprised of about 300 grams per liter of nickel sulfate, about 30 grams per liter of boric acid, and has a pH of about 1.5.

5. The process which comprises electrodepositing nickel by passing an electrodepositing current from an insoluble anode immersed in an aqueous nickel sulfate plating electrolyte substantially devoid of chloride ion and having a pH of about 0.75 to 3.5 to a cathode likewise immersed in said electrolyte to electrodeposit nickel at said cathode, flowing said electrolyte to a replenishing unit, replenishing the nickel content of said plating electrolyte in said

replenishing unit by flowing therethrough between nickel electrodes direct current at a current density of about 1 to 25 amperes per square foot from a source of reversible direct current while reversing the direction of said direct current at

intervals of about 1 to 50 seconds, flowing the thus-replenished electrolyte to an electrodepositing unit comprising an insoluble anode and a cathode and electrodepositing nickel from the thus-replenished electrolyte.

6. The process for electrodepositing nickel which comprises establishing an aqueous nickel plating electrolyte essentially comprised of about 100 to 400 grams per liter of nickel sulfate, about 10 to 50 grams per liter of boric acid, substantially devoid of chloride ions, having a pH of about 0.75 to 3.5 and a temperature of about 100° to 160° F., electrodepositing nickel from said electrolyte in an electroplating unit having a source of direct current, at least one insoluble

anode and at least one cathode by passing a plating current from said direct current source through said electrolyte from said insoluble anode to said cathode to electrodeposit nickel at said cathode, flowing said electrolyte to a replenishing unit comprising a source of reversible direct current in electrical connection with a plurality of electrolytic nickel electrodes, substantially replenishing the nickel content of said plating electrolyte by passing therethrough between said

electrodes direct current from said source of reversible direct current at a current density of about 1 to 25 amperes per square foot while repeatedly reversing the direction of said direct current at time intervals of about 1 to 50 seconds to obtain a net gain of nickel dissolved from said electrodes, flowing the thus-replenished electrolyte to an electroplating unit and electrodepositing nickel from the thus-replenished electrolyte.

7. The process according to claim 6 wherein the aqueous nickel plating electrolyte is essentially comprised of about 250 to 350 grams of nickel sulfate per liter, about 20 to 40 grams of boric acid per liter, and has a pH of about 1 to

2, and wherein the direct current in the re-

75

## 11

plenishing unit flows at a current density of about 5 to 15 amperes per square foot and the direction of said current is reversed at intervals of about 3 to 7 seconds.

8. The process according to claim 7 wherein the current in the replenishing unit flows at a current density of about 10 amperes per square foot and wherein the direction of said current is reversed at intervals of about 5 seconds.

9. The process according to claim 8 wherein the aqueous nickel plating electrolyte is essentially comprised of about 300 grams of nickel sulfate per liter, about 30 grams of boric acid per liter, and has a pH of about 1.5.

10. The process for electrodepositing nickel which comprises alternately subjecting to an electroplating operation and to a replenishing operation an aqueous nickel plating electrolyte containing about 100 to 400 grams of nickel sulfate per liter of electrolyte, about 10 to 50 grams per liter of boric acid, having a pH of about 0.75 to 3.5 and being substantially devoid of chloride ions, said electroplating operation comprising passing a plating current through said electrolyte between an insoluble anode and a cathode immersed therein to electrodeposit nickel at said cathode, said replenishing operation being conducted in a replenishing unit having a plurality of electrolytic nickel electrodes in electrical connection with a source of reversible direct current and comprising passing through said electrolyte between said electrodes direct current from said source of reversible direct current at a current density of about 1 to 25 amperes per square foot while reversing the direction of flow of said direct current at least once at intervals of about 1 to 50 seconds to obtain

in said electrolyte a net gain of nickel dissolved from said electrodes.

11. The process according to claim 10 wherein the aqueous nickel plating electrolyte is essentially comprised of about 250 to 350 grams of nickel sulfate per liter, about 20 to 40 grams of boric acid per liter, and has a pH of about 1 to 2.

EDWARD JUDSON ROEHL.  
ANDREW WESLEY.

## REFERENCES CITED

The following references are of record in the file of this patent:

## UNITED STATES PATENTS

| Number    | Name             | Date           |
|-----------|------------------|----------------|
| 1,003,092 | Dow et al.       | Sept. 12, 1911 |
| 1,144,680 | Allers           | June 29, 1915  |
| 1,885,148 | Smith            | Nov. 1, 1932   |
| 2,431,949 | Martz            | Dec. 2, 1947   |
| 2,449,422 | Smith            | Sept. 14, 1948 |
| 2,449,495 | Lum              | Sept. 14, 1948 |
| 2,451,341 | Jernstedt        | Oct. 12, 1948  |
| 2,470,775 | Jernstedt et al. | May 24, 1949   |

## FOREIGN PATENTS

| Number  | Country       | Date          |
|---------|---------------|---------------|
| 310,099 | Great Britain | Apr. 25, 1929 |
| 49,384  | Denmark       | Oct. 15, 1934 |

## OTHER REFERENCES

Transactions of the Electrochemical Society, Watts, vol. 59 (1931), page 381.

Blum et al., Transactions of the Faraday Society, vol. 31 (1935), page 1208.

Finch et al., Transactions of the Faraday Society, vol. 33 (1937), page 566.